

Sept. 11, 1945.

H. F. FRUTH

2,384,541

CONDENSER MATERIAL AND METHODS OF MAKING SAME

Filed May 5, 1942

FIG. 1



FIG. 2



FIG. 3

INVENTOR  
H. F. FRUTH  
BY Harry L. Draft  
ATTORNEY

## UNITED STATES PATENT OFFICE

2,384,541

CONDENSER MATERIAL AND METHOD OF  
MAKING SAME

Hal F. Fruth, Elmhurst, Ill., assignor to Western  
Electric Company, Incorporated, New York,  
N. Y., a corporation of New York

Application May 5, 1942, Serial No. 441,870

5 Claims. (Cl. 117—17)

This invention relates to condensers and to a method of and apparatus for making the same, and more particularly to condenser materials having oriented crystalline structure and to a method of and apparatus for making the same.

Condensers have been made by impregnating or by coating a dielectric material on a base such as paper, the dielectric material being suspended or dissolved in a binder containing a solvent which evaporates after coating or impregnating is completed.

An object of the present invention is to provide an improved condenser material having a high dielectric constant and a method of and apparatus for making the same.

In accordance with one embodiment of this invention, titanium dioxide crystals suspended in a liquid binder are coated on a strip of paper, and the coated paper is passed through an electrostatic field causing the crystals to orient their major axes perpendicular to the paper base. The coated paper is then calendered to increase its density.

In accordance with another embodiment of the invention, a quantity of titanium dioxide crystals suspended in a liquid binder are poured on a tray of volatile material and an electrostatic field applied to orient the crystals along their major axes and parallel to each other. As the binder solvent evaporates, the binder hardens and the oriented crystals become permanently fixed in their oriented position. The tray and contents may then be placed in an oven to volatilize and remove the tray and also to fire the titanium dioxide to produce a ceramic body, the crystals of which will have their major axes substantially parallel.

Other objects and advantages will be apparent from the following detailed description taken in conjunction with the following drawing, wherein:

Fig. 1 shows schematically an apparatus for coating strip material with a dielectric;

Fig. 2 shows schematically an apparatus for making sheets of dielectric material; and

Fig. 3 shows an enlarged fragmentary perspective view of an electrostatic plate such as may be used with the apparatus shown in Fig. 1.

As may be seen in Fig. 1, a base material 5 such as a paper strip or aluminum foil is drawn from a supply reel 6 over a small roller 7 and into a tank 8 containing a quantity of dielectric material 9. This material may be titanium dioxide crystals or other dielectric material possessing similar polar characteristics such as zirconium dioxide, or certain titanates and zirconates such as lead titanate, strontium titanate, lead zircon-

ate, strontium zirconate and various mixtures of two or more of these compounds. The dielectric material is suspended in a liquid binder such as cellulose acetate using acetone as a solvent, or an aqueous solution of sodium silicate. Polyvinyl alcohol may also be employed and since it is itself polar and posses desirable dielectric characteristics, its use results in even greater dielectric constant. It will be apparent that if aluminum foil is used as a support, a coating only is obtained, whereas with porous material, such as certain types of paper, impregnation may also take place. However, with the types of paper commonly used in condensers as base material, impregnation by the dielectric material is negligible.

Titanium dioxide crystals have a dielectric constant of 89 parallel to their smaller axis and 173 parallel to their major axes and about 115 for random orientation and will orient themselves in the presence of an electrostatic field so that their major axes are substantially parallel. By orienting the random crystals of a dielectric material comprising one or more of these above-mentioned compounds, a condenser material having increased dielectric constant as compared to a condenser material in which the crystals are random oriented, may be obtained. At the same time, since the crystals are aligned along the line of lowest dielectric loss, a reduction in power factor is also obtained.

The base material to be coated may be passed around a roller 10 positioned beneath the liquid in the tank. The coated or impregnated strip is then drawn from the coating bath and passed between two spaced electrical conducting plates 12 which are connected to a source of potential such as an alternating current or direct current generator 13. The charged plates preferably extend downwards as close to the liquid in the tank as practical so that the orienting force of the electrostatic field will be exerted while the crystals are most easily movable, that is, while the binder is most fluent. Since crystals align themselves in the presence of an electrostatic field along the line of lowest dielectric loss, the titanium dioxide crystals will be oriented with their major axes substantially perpendicular to the supporting strip and substantially parallel to each other. It should be noted that the major axis of a titanium dioxide crystal is not necessarily the physically longer axis, but is, as defined, the line of lowest potential energy.

Either alternating current or direct current may be used; however, alternating current or pulsating direct current has the desirable effect of jar-

ring or jolting the crystals into position whereas ordinary direct current merely exerts a constant force. This jarring or jolting appears to produce more complete orientation of the crystals.

The evaporation of the solvent and hardening of the binder may be expedited by applying heat to the strip as it is drawn between the charged plates. Preferably, the heat is applied by an oven 14 positioned so that the charged plates extend below an entrance 15 to the oven a sufficient distance to orient the crystals of dielectric material substantially completely prior to entering the oven. The plates are long enough, however, to extend into the oven a sufficient distance to maintain the crystals in oriented position until the binder has hardened enough to prevent loss of orientation. Heat may be supplied by a number of electric coils 16 inside the oven, or by gas or hot air.

It has been found that it is possible to reduce the thickness of the coated base material by calendering without materially affecting the orientation of the dielectric crystals. If the thickness of the dielectric material and base is reduced, the capacitance of the condenser is increased proportionately. This result obtains regardless of the original thickness of the dielectric material and support. At the same time the density of the dielectric material is increased, which also results in increased capacity, since more dielectric material is thereby compacted into a given space. A further advantage of calendering lies in the fact that the surface of the dielectric is rendered smoother and more resistant to abrasion. The coated, or impregnated, strip is therefore passed over a pair of rollers 17 and 18 and between a pair of steel calendering rolls 19 and 20. The strip is finally wound on a take-up reel 21.

By calendering it is possible to reduce the thickness of sheets of coated base material by approximately 30 to 45%, thus increasing the density of the dielectric material approximately 43 to 82%. This increase in density produces, as stated above, a corresponding increase in capacitance of the condenser with which the dielectric material is used. A coated sheet of .001" thickness is desirable as an ultimate size. By calendering, it is possible to obtain a sheet of this size from a coated sheet originally .0016". However, coated sheets as thick as .0020" have been successfully calendered and used as condenser materials, and calendered sheets as thin as .0008" have been successfully used as condenser materials. The amount of widening of the sheet during calendering is negligible.

In Fig. 2 another embodiment of this invention is shown. Here, instead of coating dielectric material on a strip, a quantity of dielectric material 25, which may be titanium dioxide suspended in an aqueous solution of sodium silicate, or any other suitable liquid dielectric binder as previously described, is poured onto a tray 26 or platter of easily volatile, combustible or soluble material, such as polystyrene, or of non-porous material such as glass. An electrostatic field is applied to the material by positioning an electrical conducting plate 27 above, or in contact with, the liquid and a similar plate 28 below the tray. The plates are connected to a source of potential 29, which, as previously described, may be alternating current or direct current, or pulsating direct current. The crystals are thereby oriented with their major axes substantially parallel and as the binder dries and hardens, they become fixed in position. If a polystyrene tray is used, the tray

5 may then be placed in an oven and heated sufficiently to volatilize the polystyrene and to fire the titanium dioxide, thus leaving a sheet of ceramic dielectric material, the crystals of which are oriented along their major axes and fused together. If a glass tray is used, the dielectric material may be removed from the tray and then fired. This method is feasible only when the dielectric material has considerable flexibility and may be 10 handled without breaking. By dispensing with a base material, a dielectric body of minimum dimensions is obtained. This economy of dimensions makes possible increased capacitance per given volume of condenser.

15 Some increase in the effectiveness of the potential applied to the plates used in the first of the above described embodiments of this invention may be obtained by providing each plate with a number of relatively small cone shaped points 30, as shown in Fig. 3, of conducting material, such as used for the plates, attached to one side of each plate in rows spaced about  $\frac{1}{8}$  to  $\frac{1}{4}$  of an inch apart. The points on one plate face the points on the other and the rows of points are 20 staggered so that all portions of a strip passing between the plates are subjected substantially equally to the concentrated charge at the points. By concentrating the potential in this way, a higher effective potential is obtained between the plates without increasing the voltage supplied to the plates or the net potential between the plates. High potential is desirable because the degree of orienting force exerted on the crystals is 25 directly proportional to the potential gradient.

30 While but two embodiments of this invention have been shown and disclosed, it will be understood that many changes and alterations may be made therein without departing from the spirit and scope of the present invention.

35 What is claimed is:

1. A dielectric body having high dielectric constant comprising a base having a coating of titanium dioxide particles, said particles having a higher dielectric constant along one axis than 40 along another axis and said particles being oriented so that the major electrical axes of said particles are substantially perpendicular to the base so as to increase the effective dielectric constant of said body, and a binder of a solidifiable film forming type to bond said particles in oriented position.

45 2. A dielectric body having high dielectric constant comprising a base having a coating of particles selected from the group consisting of titanates and zirconates, said particles having a higher dielectric constant along one axis than along another axis and said particles being oriented so that the major electrical axes of said particles are substantially perpendicular to the base so as to increase the effective dielectric constant of said body, and a binder of a solidifiable film forming type to bond said particles in oriented position.

50 3. A method of making a dielectric body comprising coating a base of metal foil with particles 55 of dielectric material selected from the group consisting of titanates, zirconates, titanium dioxide, and zirconium dioxide, and suspended in a solidifiable liquid binder of film forming material containing a volatile solvent, said particles having a higher dielectric constant along their major electrical axis than along their minor electrical axis, orienting said particles by applying an electrostatic field thereto so that their major electrical axes are substantially perpendicular to said

base material, and solidifying said binder by evaporating said volatile solvent.

4. A method of making a dielectric body comprising coating a base of metal foil with particles of dielectric material suspended in a solidifiable liquid binder of sodium silicate containing a volatile solvent, said particles being selected from the group consisting of titanates, zirconates, titanium dioxide and zirconium dioxide and being orientable along one axis to increase the effective dielectric constant of the body, orienting said particles by applying an electrostatic field thereto so that the major electrical axes of said particles are substantially perpendicular to the base, and evaporating said volatile solvent to solidify said binder. 15

5. A dielectric body having a high dielectric constant comprising a base having a coating of particles selected from a group consisting of titanates, zirconates, titanium dioxide and zirconium dioxide, said particles having a higher dielectric constant along one axis than along another axis and being oriented so that their major electrical axes are substantially perpendicular to the base so as to increase the effective dielectric constant of the body, and a binder of a solidifiable film forming type to bond said particles in oriented position.

HAL F. FRUTH.